

# UNITED STATES PATENT OFFICE.

ALBERT CHAMPION AND TAIN G. McDUGAL, OF FLINT, MICHIGAN, ASSIGNEES  
TO CHAMPION IGNITION COMPANY, OF FLINT, MICHIGAN, A CORPORATION OF  
MICHIGAN.

## INSULATING MATERIAL AND BODY COMPOSED THEREOF.

1,262,305.

Specification of Letters Patent.

Patented Apr. 9, 1918.

No Drawing.

Application filed August 22, 1917. Serial No. 187,581.

To all whom it may concern:

Be it known that we, ALBERT CHAMPION and TAIN G. McDUGAL, citizens of the Republic of France and the United States 5 of America, respectively, and residents of Flint, county of Genesee, State of Michigan, have invented certain new and useful Improvements in Insulating Material and Body Composed Thereof, of which the following is a specification.

Our invention relates to the manufacture of spark plugs designed for use with internal combustion engines, and particularly to the insulating members used in and forming 15 a part of such devices. One object of our invention is to provide an insulating member which will have improved dielectric strength, under the high temperature conditions present in internal combustion engines 20 and will possess a structure which will enable it to better resist sudden changes in temperature without cracking.

With the above and other objects in view, our invention consists: First: in an insulating member for the purpose stated in which the proportion of clay to the other ingredients used in the finished member and upon which its insulating properties depend, is increased, and in which the proportion of 25 those substances which have to be mixed with the clay in the practical manufacture of insulators (and which ordinarily have a deleterious effect thereupon so far as concerns the insulating properties, when used 30 at higher temperatures, of the finished product), is reduced to a minimum. Second: in an insulating member which, during the manufacture thereof is subjected to a higher firing temperature than has heretofore been 35 usual, made necessary by the new proportioning of the ingredients used in order to maintain a vitrified structure. Third: in such other improvements in and relating to insulating members for spark plugs as will 40 hereinafter appear.

Our invention not only includes an insulating member for a spark plug as a new article of manufacture, the same being made from a plastic composition made up of certain materials hereinafter enumerated, but it also includes the porcelain material *per se* 45 made from the composition or mixture disclosed, which material is capable of use

wherever high insulating qualities at high temperatures are desirable in an article or 55 device to be made therefrom, and the method or process of making insulating members for spark plugs from a composition made up of the ingredients specified, by subjecting the same to suitable operations during and 60 as steps in the manufacture of the said members from the composition disclosed.

The insulating members of spark plugs for use in internal combustion engines are ordinarily formed from a composition comprising 65 plastic clay or kaolin mixed with a certain portion of non-plastic and more or less fusible materials and molded or shaped into proper form, and then dried, and finally subjected to a high temperature, or fired, to 70 vitrify the mass. The plasticity of the mass is made possible on account of its raw clay content.

The non-plastic material (ordinarily ground flint and feldspar) is employed to 75 reduce and control the shrinkage of the molded members and to prevent the formation of cracks therein during the drying thereof at a comparatively low temperature, and before they are subjected to the firing 80 process, during which the uncombined water is driven off (but not the water held in chemical combination in the clay) also to prevent abnormal shrinkage and distortion during the vitrifying process. Fusible material (ordinarily feldspar) is used to promote 85 vitrification of the mass during the firing process, thus producing a hard, strong and compact finished product, the feldspar being melted at a lower temperature than 90 any of the other ingredients.

The less the quantity of the more fusible material present in the mixture from which the insulating members are formed, the greater will be the temperature necessary to 95 accomplish the vitrification of the mass of which the fusible material is an ingredient. This vitrified state of the finished product is necessary in order that the insulation be impervious to oil and to reducing gases present under conditions of its use. Furthermore the presence of feldspar is found to be deleterious in insulating members for spark plugs because it reduces the insulating properties thereof at the higher temperatures. 100 105

It therefore follows that a minimum

amount of feldspar is desirable, because of its direct effect in reducing the insulating qualities at higher temperatures of the finished insulator, due to its mere presence, and because vitrified bodies obtained (usually at lower heats) through high feldspar content have been found to poorly resist breakage under suddenly varying temperatures.

It is found in practice that a quantity of raw clay equal to about sixty per cent. of the composition or mixture employed should be used in order to secure the requisite plasticity to permit the various molding, lathing, kneading and other operations necessary to give the proper shape and form to the insulators, while a quantity of feldspar equal to about ten per cent. or as little as five per cent. of the composition will be sufficient to secure a proper vitrification thereof when they are subjected to the correct firing process and will at the same time not seriously lower the insulating qualities of the insulators. This quantity has been found to secure the best balance between an unavoidable impairment of insulating qualities in the finished product due to the presence of feldspar therein on the one hand, and the necessity for an excessively high firing temperature due to an inordinate reduction of the quantity of feldspar used on the other.

From the above it will be appreciated that there remains an unassigned quantity equal to 40% of the composition from which the insulators are made, which deficiency is supplied by the non-plastic materials hereinbefore referred to, as it has been found in practice that non-plastic material to the extent of about 40% of the composition is necessary to prevent cracking and undue shrinkage of the molded and shaped insulating members during the drying operation or step to which they are subjected before firing. If flint, alone, is used to make up 30% or 35% of this 40% then the fired insulators would not be uniform or homogeneous in structure, the flint being present in much the same condition as when introduced, because the flint is but slowly soluble in the molten feldspar during the firing operation.

Our invention, therefore, contemplates the use of calcined clay as the non-plastic ingredient of the composition employed for making the insulating members, either alone or in connection with a much smaller quantity of flint than the thirty or thirty-five per cent. referred to above. It follows that the amount of flint in the finished product is greatly reduced and the amount of clay upon which substitution the insulating qualities at increased temperatures of the members is dependent is proportionately increased. For example, and still assuming the 60% proportion of raw or uncalcined

clay and 10% of feldspar, then if 20% of calcined clay is used the amount of flint is reduced to 10%; and if calcined clay and feldspar alone are used as the non-plastic constituents of the composition, then the flint is eliminated altogether.

It will be appreciated that the calcined clay is produced by heating raw or ordinary plastic clay to such a temperature that the chemically combined water held therein is driven off. This heat treatment of the clay causes it to lose its plastic qualities and to become an inert or non-plastic substance. As this clay will not thereafter combine with water, the uncombined water, which is ordinarily contained in the uncalcined clay, and is therefore present in the ingredients employed, will facilitate the operations necessary to give the proper form to the insulating members before drying and firing.

Finally both the raw or uncalcined clay and the calcined clay are in precisely the same condition, and are in all respects alike after the firing process has been performed, so that the finished insulating members made in accordance with our invention are made up entirely of clay vitrified by the use of say 10% or less each of feldspar and flint, if flint is used at all.

In making an insulator for spark plugs in accordance with our invention the proper quantities of raw or uncalcined clay, calcined clay (and flint or other non-plastic material if any such is used) and feldspar, are mixed and ground together in any suitable grinding mill until the proper degree of fineness is obtained and an intimate mixture has been secured. After grinding the insulating members are properly formed from the mixture by any suitable molding, shaping, forming or similar operations. The said members are next dried at a comparatively low temperature to eliminate the water held in mechanical suspension in the composition from which they are formed, and which was either present in the raw clay or was added during the operations anterior to the final production of the formed insulating members in order to facilitate the working of the composition.

The body is then fired at the required temperature which exceeds by 40° centigrade or more that used in common porcelain manufacture.

Having thus described and explained our invention, we claim and desire to secure by Letters Patent:

1. As a new article of manufacture, an insulating member for a spark plug made from porcelain, and in which calcined clay is used as a non-plastic ingredient of the composition from which the said member is formed.

2. As a new article of manufacture, an insulating member for a spark plug formed

from a mixture containing plastic uncalcined clay, non-plastic calcined clay, and a fusible vitrifying material.

3. As a new article of manufacture, an insulating member for a spark plug formed from a mixture containing plastic uncalcined clay, non-plastic calcined clay, and feldspar.

4. As a new article of manufacture, an insulating member for a spark plug formed from a mixture comprising plastic uncalcined clay, a non-plastic material made up of calcined clay and flint, and a fusible vitrifying material.

5. As a new article of manufacture, an insulating member for a spark plug formed from a mixture comprising plastic uncalcined clay, a non-plastic material made up of calcined clay and flint, and feldspar.

6. As a new article of manufacture, an insulating member for a spark plug formed from a mixture comprising approximately 60% of plastic uncalcined clay, approximately 10% of a fusible vitrifying material, and approximately 30% of non-plastic material some of which is calcined clay.

7. As a new article of manufacture, an insulating member for a spark plug formed from a mixture comprising approximately 60% of plastic uncalcined clay, approximately 10% of feldspar, and approximately 30% of non-plastic material some of which is calcined clay.

8. The insulating material herein described and made from a mixture comprising approximately 60% of plastic uncalcined clay, approximately 10% of fusible vitrifying material, and approximately 30% of non-plastic material some of which is calcined clay. 35

9. The insulating material herein described and made from a mixture comprising approximately 60% of plastic uncalcined clay, approximately 10% of a fusible vitrifying material, and approximately 30% of non-plastic material made up of calcined 40 45 clay and flint.

10. The insulating material herein described and made from a mixture comprising approximately 60% of plastic uncalcined clay, approximately 10% of feldspar, and approximately 30% of non-plastic material 50 some of which is calcined clay.

11. The insulating material herein described and made from a mixture comprising approximately 60% of plastic uncalcined clay, approximately 10% of feldspar, and approximately 30% of non-plastic material 55 made up of calcined clay and flint.

In witness whereof we have hereunto set 60 our hands at Flint, county of Genesee, State of Michigan, this 17th day of August, 1917.

ALBERT CHAMPION.  
TAINE G. McDUGAL.